

# United States Patent [19]

Tanaka et al.

[11] Patent Number: 4,707,427

[45] Date of Patent: Nov. 17, 1987

[54] **SQUARYLIUM COMPOUND IN AN ELECTROPHOTOGRAPHIC ELEMENT**

[75] Inventors: Hiroyuki Tanaka; Seki Kin; Lyong S. Pu, all of Kanagawa, Japan

[73] Assignee: Fuji Xerox Co., Ltd., Tokyo, Japan

[21] Appl. No.: 946,641

[22] Filed: Dec. 29, 1986

### Related U.S. Application Data

[60] Continuation of Ser. No. 744,853, Jun. 14, 1985, abandoned, which is a division of Ser. No. 682,211, Dec. 17, 1984, Pat. No. 4,700,001.

[30] **Foreign Application Priority Data**

Dec. 16, 1983 [JP] Japan ..... 58-236201

Dec. 21, 1983 [JP] Japan ..... 58-239815

Dec. 21, 1983 [JP] Japan ..... 58-239816

[51] Int. Cl.<sup>4</sup> ..... G03G 5/06; G03G 5/14

[52] U.S. Cl. ..... 430/59; 430/58; 430/73; 430/74; 564/307

[58] **Field of Search** ..... 430/58, 59, 73, 74; 564/307

[56] **References Cited**

### U.S. PATENT DOCUMENTS

4,391,888 7/1983 Chang et al. ..... 430/58 X  
4,508,803 4/1985 Law et al. ..... 430/59 X

4,523,035 6/1985 Yanus ..... 564/307  
4,628,018 12/1986 Lin et al. ..... 430/59

*Primary Examiner*—Roland E. Martin  
*Attorney, Agent, or Firm*—Sughrue, Mion, Zinn,  
Macpeak & Seas

[57] **ABSTRACT**

Novel squarylium compounds, a process for the production thereof as well as to a photoreceptor for electrophotography containing the squarylium compound are disclosed, said squarylium compounds being represented by formula (I):



wherein R is a straight-chain alkyl group having 2 or more carbon atoms or  $-\text{C}_2\text{H}_4\text{X}$ , wherein X is a hydroxyl group, a halogen atom or the group  $-\text{OR}_1$  wherein  $\text{R}_1$  is an alkyl group having 1 to 6 carbon atoms, or a substituted or unsubstituted phenyl group.

**24 Claims, 3 Drawing Figures**

FIG. 1



FIG. 2



FIG. 3



## SQUARYLIUM COMPOUND IN AN ELECTROPHOTOGRAPHIC ELEMENT

This is a continuation of application Ser. No. 744,853, now abandoned filed 6-14-85, which is a divisional of application Ser. No. 682,211 filed 12/7/84, now U.S. Pat. No. 4,700,001.

### FIELD OF THE INVENTION

The present invention relates to a novel squarylium compound and a process for the production thereof, as well as to a photoreceptor for electrophotography containing the squarylium compound.

### BACKGROUND OF THE INVENTION

Common photoreceptors for use in electrophotography are inorganic light-sensitive materials such as amorphous selenium, selenium compounds, cadmium sulfide and zinc oxide, as well as organic compounds typified by poly(vinylcarbazole) and poly(vinylcarbazole) derivatives.

As is well known, amorphous selenium and selenium alloys have excellent properties for use as electrophotographic photoreceptors and are commercially used. However, their manufacture requires the complex step of vapor deposition, and the vapor deposited film has no flexibility. Zinc oxide as a photoreceptor material is dispersed in a resin to prepare a disperse light-sensitive composition, but this has low mechanical strength and is not suitable for cyclic use.

Poly(vinylcarbazole) widely known as an organic photoconductive material is advantageous with respect to transparency, film-forming properties and flexibility. However, poly(vinylcarbazole) per se is insensitive to light in the visible range and cannot be immediately used as a photoreceptor. Various methods have been proposed for sensitizing the poly(vinylcarbazole). The use of a sensitizing dye is effective in extending the spectral sensitivity of the poly(vinylcarbazole) to the visible range, but the sensitivity of the so treated polyvinyl carbazole is still insufficient for use as an electrophotographic photoreceptor and it undergoes significant fatigue under light illumination. When poly(vinylcarbazole) is chemically sensitized with an electron acceptor compound, sufficient sensitivity for use as an electrophotographic photoreceptor is obtained. Several of the so treated poly(vinylcarbazole) compounds are commercially used, but their mechanical strength and service life are still unsatisfactory.

Among photoreceptors having sensitivity to light in the longer wavelength region are inorganic compounds such as Se/Te, Se/As and CdSe. Many of these inorganic compounds are designated as poisons, dangerous drugs or special chemical substances under regulations that require utmost care in handling, particularly in disposal. Furthermore, these compounds are difficult to manufacture and their production cost is high. As another disadvantage, they have no flexibility and can only be shaped into a belt form with great difficulty.

Energetic efforts have been made in the study of electrophotographic photoreceptors using organic disperse photosensitive materials wherein a charge generation layer and a charge transport layer are laminated on an electrically conductive support. For example, U.S. Pat. No. 4,018,953 discloses an electrophotographic photoreceptor having a charge generation layer containing an organic photoconductive materials such as

phthalocyanine type pigments, quinacridones, etc. and a charge transport layer having a specific aromatic diamine dispersed in a binder (hereafter referred to as "double-layered photoreceptor"). Double-layered photoreceptors using other organic disperse photosensitive materials are also described in U.S. Pat. Nos. 4,050,935, 4,127,412, 4,173,472, 4,175,960 and 4,284,699. Several authors have reported that phthalocyanine in the form of a disperse photosensitive material exhibits excellent electrophotographic characteristics (U.S. Pat. Nos. 4,018,953 and 4,181,772). Organic phthalocyanine compounds are non-toxic and inexpensive, but they have low sensitivity to light below 550 nm and are difficult to purify. No practical phthalocyanine compound has been found that exhibits flat photosensitivity characteristics over the visible to near infrared region.

U.S. Pat. No. 3,824,099 discloses a double-layered photoreceptor having a charge generation layer containing squaric acid pigments dispersed in a binder and a charge transport layer of tri-aryl pyrazoline, and U.S. Pat. No. 4,123,270 discloses a photoreceptor having a charge generation layer containing derivatives of squaric acid pigments which are soluble in an organic primary amine. The squaric acid pigments used in these U.S. patents are represented by the formula



wherein B is



and Z is a hydrogen atom, a hydroxy group or a methyl group. However, these squaric acid pigments still have defects in that charge retention is low and residual potential is high, resulting in low image density and high fog density. Further, the squaric acid pigments do not exhibit flat photosensitivity characteristics over the visible to near infrared region.

### SUMMARY OF THE INVENTION

One object of the present invention is to provide an extremely highly sensitive photoconductive material that can be used with any of the existing electrophotographic processes and which has spectral sensitivity over the visible to infrared region, high charge retention and low residual potential.

A second object of the invention is to provide a process for the production of this photoconductive material.

Another object of the present invention is to provide a highly sensitive and mechanically strong (e.g., high wear resistance) photoreceptor for electrophotography that is free from the defects (i.e., low wear resistance and insufficient mechanical strength) of a poly(vinylcarbazole)trinitrofluorenone type light-sensitive material

and which has substantially flat spectral sensitivity characteristics extending from the visible to near infrared region.

The present inventors have made various studies to obtain a photoconductive material that is free from the defects of the conventional inorganic photosensitive materials, organic photosensitive materials and organic disperse photosensitive materials and which instead have excellent electrophotographic characteristics and flexibility, and which exhibit high sensitivity over a wide range covering the visible and near infrared wavelengths. As a result, the inventors have found that the above objects are attained by novel squarylium compounds represented by the following formula (I):



15

20

25

30

35

40

45

50

55

60

65

65

70

75

80

85

90

95

100

ably 120°–140° C. The solvent may be used as admixture with a low boiling point solvent (e.g., benzene, toluene, etc.). If the reaction temperature is more than 150° C., the reaction products may be decomposed. The resulting compound is washed and purified by recrystallization from a suitable solvent.

Specific examples of the so prepared novel squarylium compound of formula (I) of the present invention are identified below by their structural formulae, although the present invention is not to be construed as being limited thereto.

wherein R is a straight chain alkyl group having 2 or more carbon atoms or  $-\text{C}_2\text{H}_4\text{X}$ ; and X is a hydroxy group, a halogen atom or the group  $-\text{OR}_1$  wherein  $\text{R}_1$  is an alkyl group having 1 to 6 carbon atoms or a substituted or unsubstituted phenyl group.

The squarylium pigment of formula (I) is obtained by reacting 3,4-dihydroxy-3-cyclobutene-1,2-dione of formula (II) (hereinafter referred to as "squaric acid"):



15

20

25

30

35

40

45

50

55

60

65

70

75

80

85

90

95

100

with an aniline derivative of formula (III):



15

20

25

30

35

40

45

50

55

60

65

70

75

80

85

90

95

100

wherein R is the same as defined in general formula (I).

#### BRIEF DESCRIPTION OF THE DRAWINGS

FIGS. 1 and 2 are cross sections of illustrative layer arrangements of the electrophotographic photoreceptor of the present invention.

FIG. 3 is a graph showing sensitivity curve of the photoreceptor produced in Example 4.

#### DETAILED DESCRIPTION OF THE INVENTION

In general formula (I) the halogen atom for X is preferably a fluorine atom, a chlorine atom or a bromine atom. The straight-chain alkyl group for R preferably has not more than 6 carbon atoms and more preferably not more than 4 carbon atoms.

In the process according to the invention, the compounds represented by general formula (I) are obtained by reacting squaric acid with the aniline derivative in a solvent (e.g., n-butanol or amyl alcohol) for about 3–5 hours at a temperature of not more than 150° C., prefer-

|    | Structural formula | Compound No. |
|----|--------------------|--------------|
| 15 |                    | (1)          |
| 20 |                    | (2)          |
| 25 |                    | (3)          |
| 30 |                    | (4)          |
| 35 |                    | (5)          |
| 40 |                    | (6)          |
| 45 |                    | (7)          |

Processes for producing the novel squarylium compounds of the present invention are described by the following synthesis examples, although the present invention is not to be construed as being limited thereto.

#### SYNTHESIS EXAMPLE 1

(Preparation of Compound (1))

N-Ethyl-N-methylaniline (2.37 g) and 3,4-dihydroxy-3-cyclobutene-1,2-dione (1 g) were added to a mixed solution of n-butanol (70 ml) and benzene (10 ml). The

resulting mixture was heated at an oil bath temperature of 120°–130° C. for 4 hours under agitation. After cooling, the resulting green crystal was collected by filtration, washed with methanol, and dried to obtain 1.2 g of the desired squarylium compound (1) in a yield of 39.1%. Analysis of compound (1) revealed the following characteristics:

Decomposition point: 219° C.

IR absorption spectrum (KBr tablet):  $\nu_{C=O} = 1580$  cm<sup>-1</sup>.

| Elemental analysis: |        |            |
|---------------------|--------|------------|
|                     | Found  | Calculated |
| C                   | 75.86% | 75.83%     |
| H                   | 7.00%  | 6.94%      |
| N                   | 8.21%  | 8.04%      |

Visible light absorption spectrum:  $\lambda_{max} = 634$  nm (in dichloromethane).

### SYNTHESIS EXAMPLES 2 AND 3

(Preparation of Compounds (2) and (3))

In the same manner as in Synthesis Example 1, the reaction between 3,4-dihydroxy-3-cyclobutene-1,2-dione and the aniline derivative was performed, using the different aniline derivatives shown in Table 1. Table 1 shows data on the compounds produced in Synthesis Examples 2 and 3 with respect to the decomposition point, IR absorption spectrum and visible light absorption spectrum. Table 2 shows the results of elemental analysis of these compounds.

TABLE 1

| Compound No. | Aniline derivative | Decomposition point | IR absorption spectrum | Visible light absorption spectrum* |
|--------------|--------------------|---------------------|------------------------|------------------------------------|
| (2)          |                    | 221° C.             | 1580 cm <sup>-1</sup>  | 635 nm                             |
| (3)          |                    | 224° C.             | 1590 cm <sup>-1</sup>  | 637 nm                             |

Note  
\*in dichloromethane

TABLE 2

| Compound No. | Molecular formula                                             | Found                          | Calculated               |
|--------------|---------------------------------------------------------------|--------------------------------|--------------------------|
| (2)          | C <sub>24</sub> H <sub>28</sub> N <sub>2</sub> O <sub>2</sub> | C 76.72%<br>H 7.38%<br>N 7.30% | 76.56%<br>7.50%<br>7.44% |
| (3)          | C <sub>26</sub> H <sub>30</sub> N <sub>2</sub> O <sub>2</sub> | C 77.55%<br>H 7.50%<br>N 7.00% | 77.58%<br>7.51%<br>6.96% |

### SYNTHESIS EXAMPLE 4

(Preparation of Compound (4))

N-Hydroxyethyl-N-methylaniline (5.3 g) and 3,4-dihydroxy-3-cyclobutene-1,2-dione (1.0 g) were added to n-butanol (35 ml). The resulting mixture was heated at 120°–130° C. for 5.5 hours under agitation. After cooling, the resulting bluish green crystal was collected by filtration, washed with methanol, recrystallized from

chloroethanol, and dried to obtain 1.3 g of the desired squarylium compound (4) (38.0%). Analysis of compound (4) revealed the following characteristics:

Decomposition point: 260° C.

IR absorption spectrum (KBr tablet):  $\nu_{C=O} = 1590$  cm<sup>-1</sup>.  $\nu_{OH} = 3370$  cm<sup>-1</sup>.

| 10 | Elemental analysis: |            |
|----|---------------------|------------|
|    | Found               | Calculated |
| C  | 69.26%              | 69.49%     |
| H  | 6.40%               | 6.36%      |
| N  | 7.21%               | 7.36%      |

15 Visible light absorption spectrum:  $\lambda_{max} = 633$  nm (in dichloromethane).

### SYNTHESIS EXAMPLES 5 TO 7

(Preparation of Compounds (5)–(7))

20 In the same manner as in Synthesis Example 4, the reaction between 3,4-dihydroxy-3-cyclobutene-1,2-dione and the aniline derivative was performed, using the different aniline derivatives shown in Table 3. Table 3 shows data on the compounds produced in Synthesis Examples 5 to 7 with respect to the decomposition point, IR absorption spectrum and visible light absorption spectrum. Table 4 shows the results of elemental analysis of these compounds.

TABLE 3

| Compound No. | Aniline derivative | Decomposition point | IR absorption spectrum | Visible light absorption spectrum |
|--------------|--------------------|---------------------|------------------------|-----------------------------------|
| (5)          |                    | 213° C.             | 1580 cm <sup>-1</sup>  | 633 nm*                           |
| (6)          |                    | 235° C.             | 1610 cm <sup>-1</sup>  | 628 nm*                           |
| (7)          |                    | 231° C.             | 1610 cm <sup>-1</sup>  | 637 nm**                          |

Note  
\*in dichloromethane  
\*\*in methanol

TABLE 4

| Compound No. | Molecular formula                                                             | Found                                       | Calculated                         |
|--------------|-------------------------------------------------------------------------------|---------------------------------------------|------------------------------------|
| (5)          | C <sub>24</sub> H <sub>28</sub> N <sub>2</sub> O <sub>4</sub>                 | C 70.24%<br>H 6.74%<br>N 7.00%              | 70.57%<br>6.91%<br>6.86%           |
| (6)          | C <sub>22</sub> H <sub>22</sub> N <sub>2</sub> O <sub>2</sub> Cl <sub>2</sub> | C 58.63%<br>H 4.82%<br>N 6.35%<br>Cl 15.52% | 58.81%<br>4.94%<br>6.23%<br>15.77% |
| (7)          | C <sub>22</sub> H <sub>22</sub> N <sub>2</sub> O <sub>2</sub> Br <sub>2</sub> | C 49.11%<br>H 4.15%<br>N 5.06%<br>Br 29.62% | 49.09%<br>4.12%<br>5.20%<br>29.66% |

65 The novel squarylium compounds thus prepared are effective for use as charge generation materials in a multilayered photoreceptor.

These compounds exhibit flat characteristics in the spectral sensitivity over the range of 400-850 nm, and they have sufficient sensitivity to light in both the visible and near infrared regions.

Therefore, the novel squarylium compounds of the present invention may be used not only with conventional electrophotographic copiers but also with semiconductor laser printers in intelligent copiers. The use of these compounds is not limited to electrophotography; they may also be used with optical recording media (e.g., laser discs) and organic solar cells.

The squarylium pigments of formula (I) can be used in multi-layered photoreceptors in electrophotography. More specifically, the squarylium pigment is incorporated in the charge generation layer of a double-layered photoreceptor, and combined with a known charge transport layer which typically is composed of a photoconductive polymer such as poly(vinyldibenzothiophene), poly(vinylpyrene), poly(vinylanthracene) or poly(vinylcarbazole), or which has triarylpypyrazoline, triphenylmethane, oxadiazole, tetraphenylbenzidine or trinitrofluorenone incorporated in a binder resin, as described in U.S. Pat. Nos. 4,018,953 and 4,150,987. The binder resin for the charge transport layer may be selected from those described later as a binder for the charge generation layer, and those described in U.S. Pat. Nos. 3,121,006, 3,870,516, 4,018,953, 4,284,699 and 4,173,472 may also be used. The so prepared photoreceptor has improved charge retention, reduced residual potential and enhanced mechanical strength.

Two typical embodiments of the double-layered photoreceptor for use in electrophotographic process are illustrated in FIGS. 1 and 2, wherein an electrically conductive support 1 is coated with a light-sensitive layer 4 composed of an assembly of a charge generation layer 2 containing the squarylium pigment and a charge transport layer 3 containing a charge transport material. The thickness ratio of the charge generation layer to the charge transport layer is preferably from about  $\frac{1}{2}$  to about 1/200. Further, the squarylium pigment and a charge transport material may be incorporated into one layer to form a single-layered photoreceptor, if desired.

The squarylium pigment in the charge generation layer may be used either alone or in combination with a suitable binder resin. In the latter case, the pigment is generally used in an amount of about 10-90 wt%, preferably about 10-50 wt%, of the charge generation layer, and the pigment is dispersed in the form of particles in the binder resin.

If the squarylium pigment alone is used, the charge generation layer may be prepared by solvent coating or vacuum vapor deposition.

The thickness of the charge generation layer generally ranges from about 0.1 to 3 $\mu$ , preferably about 0.2 to 1 $\mu$ .

For the purpose of its dispersion in a binder, the pigment may be ground into fine particles by a known method using any conventional mill, such as an SPX MILL, ball mill or RED DEVIL (trade name). Particle size of the pigment is generally not more than 5 $\mu$ , preferably 0.01 to 3 $\mu$ , but the particle size is not limited thereto.

The binder used in the charge generation layer may or may not be photoconductive by itself. Illustrative photoconductive binders are photoconductive polymers such as poly(vinylcarbazole), poly(vinylcarbazole) derivatives, poly(vinylnaphthalene), poly(vinylanthracene) and poly(vinylpyrene), as well as or-

ganic matrix materials having the charge transporting capability.

Known insulating resins having no photoconductivity may also be used as a binder. Illustrative known insulating resins include polystyrene, polyesters, poly(vinyltoluene), poly(vinylanisole), poly(chlorostyrene), poly(vinylbutyral), poly(vinyl acetate), poly(vinylbutyl methacrylate), copoly(styrene-butadiene), polysulfone, copoly(styrene-methylmethacrylate), and polycarbonates.

In order to further improve the mechanical strength of the photoreceptor, plasticizers may be used as in the case of general polymeric materials. Suitable plasticizers include chlorinated paraffin, chlorinated biphenyl, and phosphate and phthalate compounds. These plasticizers may be used in an amount of about 0-10 wt% of the binder, achieving the intended object of providing further improved mechanical strength without compromising the sensitivity or electrical properties of the receptor.

The binder having the squarylium pigment dispersed therein is coated onto the electrically conductive support. Any known coating technique such as immersion coating, spray coating, bar coating and applicator coating may be employed for the purpose of providing the desired charge generation layer.

Usable electrically conductive supports include metals (e.g., aluminum, nickel, chromium, iron, stainless, copper, etc.), paper which is rendered electrically conductive, as well as polymeric films and glass plates having an electrically conductive coat of the above metals, Au, Ag, indium oxide, indium tin oxide, etc.

A surface layer such as a protective layer and an insulating layer may further be provided on the light-sensitive layer so as to prevent mechanical damage and chemical change in properties of the light-sensitive layer. The protective layer is a layer having low electric resistance of  $10^8$  to  $10^{14}$   $\Omega$ cm which can be used in so-called Carlson process, and the insulating layer is an electrically insulating layer which can be used in a process as described in U.S. Pat. Nos. 3,401,167 and 3,438,706. Both layers are substantially transparent to light for exposure and the thicknesses of the protective layer and the insulating layer are about 2 to 20 $\mu$  and about 10 and 40 $\mu$ , respectively.

In order to prevent injection of electron from an electrically conductive support to the light-sensitive layer, a barrier layer may be formed between the support and the light-sensitive layer. For the purpose, aluminum oxide, nylon, epoxy resins can be used. Such a barrier layer may not be formed when the photoreceptor is used in the process of U.S. Pat. Nos. 3,041,167 and 3,438,706 as described above or when the charge transport layer is formed as a lower layer on the support in the preparation of double-layered photoreceptor (FIG. 2). An adhesive layer may also be formed between the support and the light-sensitive layer to improve adhesion therebetween.

The electrophotographic photoreceptor of the present invention may be used not only with ordinary copiers but also with laser printers, as well as intelligent copiers since the photoreceptor of the present invention is sensitive to laser. Laser which can be applied to the photoreceptor of the present invention is preferably a semiconductor laser such as those of Ga-As type semiconductors (e.g., Ga-As, Al-Ga-As, Ga-As-P, etc.).

Specific embodiments of the present invention are further described by reference to working examples,

which are not to be construed as limiting the scope of the invention. Unless otherwise indicated, all parts, percents and ratios are by weight, and surface potential  $V_0$  given is an absolute value.

#### EXAMPLES 1 TO 4

10 g of squarylium pigment shown in Table 5 was ground in a ball mill for 12 hours in the presence of 160 ml of methylene chloride. The ground particles (30 wt%) having an average particle size of 0.1  $\mu\text{m}$  were added to a polyester resin (tradename "Vylon 200"; weight average molecular weight 15,000) and mixed therewith. The resulting mixture was coated onto an aluminum plate by an applicator to form a charge generation layer in a dry thickness of about 0.5  $\mu\text{m}$ . A mixture of 50 wt% of 1-phenyl-3-(*p*-diethylaminostyryl)-5-(*p*-diethylaminophenyl)-pyrazoline with a polycarbonate resin (tradename "Panlite"; weight average molecular weight 28,000) was coated onto the charge generation layer by an applicator, so as to form a charge transport layer in a thickness of about 15  $\mu\text{m}$ .

The photoreceptor was mounted in a paper analyzer (product of Kawaguchi Electric Works Co., Ltd.) and charged to a negative voltage of 6 kV by corona discharge that continued for 2 seconds. The photoreceptor was then left in the dark for 2 seconds and the resulting surface potential  $V_0$  was measured. Subsequently, the photoreceptor was exposed to a tungsten halide lamp (10 lx) until the surface potential dropped to  $\frac{1}{2} V_0$ . By this procedure, the half exposure ( $E_{\frac{1}{2}}$ ) in seconds of the photoreceptor was determined. The results are shown in Table 5. Further, the photoreceptor using squarylium pigment (4) was subjected to exposure to light while increasing the wavelength from 400 to 850 nm by 50 nm, and the exposure amount and the amount of charge decay of the photoreceptor were measured in order to calculate the sensitivity to light with respect to wavelength of light. FIG. 3 shows the sensitivity curve of the photoreceptor.

TABLE 5

| Ex. No. | Pigment | R                                 | Vo (V) | E <sub>1/2</sub> (lx.sec.) |
|---------|---------|-----------------------------------|--------|----------------------------|
| 1       | (1)     | -C <sub>2</sub> H <sub>5</sub>    | 760    | 1.6                        |
| 2       | (2)     | -C <sub>3</sub> H <sub>7</sub>    | 750    | 1.8                        |
| 3       | (3)     | -C <sub>4</sub> H <sub>9</sub>    | 770    | 2.0                        |
| 4       | (4)     | -C <sub>2</sub> H <sub>4</sub> OH | 730    | 2.2                        |

### EXAMPLES 5 TO 7

Photoreceptors were prepared as in Example 1 except using squarylium pigments (5), (6) and (7) of formula (I) wherein R =  $C_2H_4OCH_3$ ,  $C_2H_4Cl$  and  $C_2H_4Br$ , respectively. The electrical properties of the three samples are shown in Table 6.

TABLE 6

| Ex. No. | Pigment | Vo (V) | E½ (lx.sec.) |
|---------|---------|--------|--------------|
| 5       | (5)     | 700    | 2.4          |
| 6       | (6)     | 750    | 1.9          |
| 7       | (7)     | 770    | 2.0          |

### EXAMPLES 8 TO 11

As in Examples 8 to 11 and using squarylium pigments (4) to (7), photoreceptors were prepared except that the charge generation layer was formed on, rather than under, the charge transport layer. The electrical properties of the samples are shown in Table 7.

TABLE 7

| Ex. No. | Pigment | $V_o$ (V) | $E_{\frac{1}{2}}$ (lx.sec.) |
|---------|---------|-----------|-----------------------------|
| 8       | (4)     | 750       | 3.4                         |
| 9       | (5)     | 720       | 3.5                         |
| 10      | (6)     | 760       | 2.2                         |
| 11      | (7)     | 800       | 3.0                         |

The photoreceptors using the squarylium pigments of the present invention exhibit flat photosensitivity characteristics over the visible to infrared region, in other words, exhibit improved sensitivity to light of infrared region. Further since the photoreceptors of the present invention possess high charge retention and low residual potential even after repeated use, high contrast electric latent image can be formed upon electrophotographic processings, resulting in the formation of image having high image density with minimized fog density and having good image reproducibility. Furthermore the squarylium pigments of the present invention is excellent with respect to non-toxicity.

25 While the invention has been described in detail and with reference to specific embodiments thereof, it will be apparent to one skilled in the art that various changes and modifications can be made therein without departing from the spirit and scope thereof.

What is claimed is:

What is claimed is:

1. A photoreceptor for electrophotography, comprising an electroconductive support and a light-sensitive layer comprising the squarylium compound of general formula (I):



wherein R is  $-\text{C}_2\text{H}_4\text{X}$ , wherein X is a hydroxyl group, a halogen atom or the group  $-\text{OR}_1$  wherein  $\text{R}_1$  is an alkyl group having 1 to 6 carbon atoms, or a substituted or unsubstituted phenyl group.

2. The photoreceptor claimed in claim 1, wherein said light-sensitive layer comprises a charge transport layer and a charge generation layer containing said squarylium compound.

3. The photoreceptor claimed in claim 2, wherein said charge transport layer comprises a photoconductive polymer selected from the group consisting of poly(-vinyldibenzothiophene), poly(vinylpyrene), poly(-vinylanthracene) and poly(vinylcarbazole).

4. The photoreceptor claimed in claim 2, wherein said charge transport layer comprises a charge transport material selected from the group consisting of triaryl-pyrazoline, triphenylmethane, oxadiazole, tetraphenylbenzidine and trinitrofluorenone and a binder resin.

5. The photoreceptor claimed in claim 2, wherein said charge generation layer is comprised substantially of said squarylium compound.

6. The photoreceptor claimed in claim 2, wherein said charge generation layer contains said squarylium compound in an amount of from about 10 to 90 weight percent based on the weight of said charge generation layer.

7. The photoreceptor claimed in claim 6, wherein said squarylium compound is present in an amount of from

about 10 to 50 weight percent based on the weight of said charge generation layer.

8. The photoreceptor claimed in claim 2, wherein said charge generation layer is from about 0.1 to 3 micron thick.

9. The photoreceptor claimed in claim 8, wherein the thickness ratio of said charge generation layer to said charge transport layer is from about  $\frac{1}{2}$  to about 1/200.

10. The photoreceptor claimed in claim 2, wherein said charge generation layer is between said support and said charge transport layer.

11. The photoreceptor claimed in claim 2, wherein said charge transport layer is between said support and said charge generation layer.

12. The photoreceptor claimed in claim 1, wherein said light-sensitive layer comprises a layer containing said squarylium compound and a charge transport material.

13. A electrophotographic photoreceptor comprising an electroconductive support having provided thereon a photosensitive layer having dispersed in the form of particles therein a squarylium compound represented by general formula (I) as a charge generation material:



wherein R is  $-C_2H_4X$ ; and X is a hydroxy group, a halogen group or the group  $-OR_1$  wherein  $R_1$  is an alkyl group having 1 to 6 carbon atoms or substituted or unsubstituted phenyl group.

14. The photoreceptor as claimed in claim 13, wherein the squarylium compound is dispersed in the form of particles of not more than  $5 \mu m$  in size.

15. The photoreceptor as claimed in claim 13, wherein the squarylium compound is dispersed in the form of particles of 0.01 to  $3 \mu m$  in size.

16. The photoreceptor as claimed in claim 13, wherein said photosensitive layer comprises a charge transport layer and a charge generation layer containing said squarylium compound.

17. An electrophotographic photoreceptor comprising an electroconductive support having provided thereon a single layered photosensitive layer containing a charge transport material and a squarylium compound which is dispersed as a charge generation material in the form of particles, said squarylium compound being represented by general formula (I):



wherein R is  $-C_2H_4X$ ; and X is a hydroxy group, a halogen group or the group  $-OR_1$  wherein  $R_1$  is an alkyl group having 1 to 6 carbon atoms or substituted or unsubstituted phenyl group.

18. The photoreceptor as claimed in claim 1, wherein said charge transport layer comprises a charge transport material selected from the group consisting of triarylpyrazoline, triphenylmethane, oxadiazole, tetraphenylbenzidine and trinitrofluorenone and a binder resin.

19. The photoreceptor as claimed in claim 16, wherein said charge generation layer comprises said squarylium compound in an amount of from about 10 to 90 weight percent based on the weight of said charge generation layer.

20. The photoreceptor as claimed in claim 19, wherein said squarylium compound is present in an amount of from about 10 to 50 weight percent based on the weight of said charge generation layer.

21. The photoreceptor as claimed in claim 16, wherein said charge generation layer is from about 0.1 to 3 micron thick.

22. The photoreceptor as claimed in claim 16, wherein the thickness ratio of said charge generation layer to said charge transport layer is from about  $\frac{1}{2}$  to about 1/200.

23. The photoreceptor as claimed in claim 17, wherein the squarylium compound is dispersed in the form of particles of not more than  $5 \mu m$  in size.

24. The photoreceptor as claimed in claim 17, wherein the squarylium compound is dispersed in the form of particles of 0.01 to  $3 \mu m$  in size.

\* \* \* \* \*